

# UNITED STATES PATENT OFFICE.

HARRY C. MCKAY, OF ESSINGTON, PENNSYLVANIA, ASSIGNOR, BY MESNE ASSIGNMENTS, TO AMERICAN PATENT KID COMPANY, A CORPORATION OF NEW JERSEY.

## VARNISH FOR MAKING ENAMEL AND PATENT LEATHERS.

SPECIFICATION forming part of Letters Patent No. 704,082, dated July 8, 1902.

Application filed December 29, 1900. Serial No. 41,461. (No specimens.)

*To all whom it may concern:*

Be it known that I, HARRY C. MCKAY, a citizen of the United States, residing at Essington, Delaware county, Pennsylvania, have 5 invented a certain new and useful Varnish for Making Enamel and Patent Leathers, of which the following is a full, clear, and exact description.

My invention relates to a preparatory varnish to be applied to the surface of a tanned or properly-prepared skin to enable it to receive and hold any usual finishing varnish commonly applied to form the exterior or enamel surface of enamel and patent leathers. 10 Heretofore patent and enamel leathers made of calfskins were usually if not entirely enameled on the flesh side of the skin; but other skins, such as sheep and kid skins, were so enameled on either side, sometimes, but not 15 always, preceded by a roughening or buffing of the grain-surface when the enamel was applied to the grain side of the skin; but on either kind of skins and no matter how prepared after tanning the enamel heretofore 20 employed formed a stiff surface, more or less lacking in pliability, liable to crack, and otherwise open to many well-known objections, and this was due largely to the fact that the 25 enamel varnish was, in effect, nothing but a thick adhering paste wholly incapable of 30 homogeneous union with the fiber of the skin, though less open to that objection when applied to the flesh side than when applied to the grain side of the skin. In the making of 35 enamel and patent leathers it has always been and still is deemed necessary to apply at least two, and more frequently three or four, coats of the enamel varnish, sometimes rubbing or 40 roughening with pumice-stone the surface of each coat preceding the last to give it a more adhesive surface.

I have discovered that if the first varnish applied to the tanned skin be a compound composed of a drying oil, specifically boiled 45 linseed-oil, and a vehicle of high penetrative and adherent power on such substance as skin-tissue, specifically a pyroxylin solution thinned with amyl acetate—that is to say, a thin varnish of high penetrating properties, in 50 which the ingredients employed are of such a

character that the varnish will thoroughly penetrate the grain-surface of the skin and tenaciously adhere to the fibers thereof—the ordinary finishing enamels commonly used in making patent and enamel leathers may be employed to produce a finished leather in which 55 there will be a substantial homogeneity in the union of enamel and skin substance to an equal extent, whether the enameling be done upon the flesh side or upon the grain side without any buffing or roughening of the surface, the employment of my preparatory varnish, applied as hereinafter described, resulting in an absence of the usual stiffness commonly inherent in finished patent and enamel leathers 60 with almost complete absence of the common tendency to crack on the surface and possessing an elasticity and pliability almost equal to common glazed kid and other light-weight 65 leathers.

My preparatory varnish is a true mordant in the sense that when applied it is instantly taken up and absorbed by the grain side of the skin, penetrating through the external surface thereof and permeating and adhering 70 to the entire fibrous structure of the grain side, forming on such fibrous structure a penetrable film or foundation surface to which the external varnish unites or at least attaches itself with remarkable tenacity, practically 75 uniting therewith.

I will now proceed to describe my new preparatory varnish, its essential ingredients, the best mode of compounding the same, and the best mode of applying it to the skin-surface. 80

One (1) quart of linseed-oil, to which a thickening and drying matter, such as one-half ( $\frac{1}{2}$ ) ounce of raw umber, is added, is boiled to the consistency of fresh mucilage or thick molasses. I thin or reduce this oil by 85 adding, according to the temperature of the weather, about an equal bulk of amyl acetate or sufficient to give the solution a consistency of 31° Baumé. I next prepare separately two (2) gallons in bulk of a solution composed of, 90 say, sixteen (16) ounces of guncotton, dissolved in about two (2) gallons of amyl acetate, and that mixture gives the bulk stated when of the consistency of fresh mucilage or 95 molasses. These two solutions are then mixed 100

together, adding to the compound a coloring pigment, say, any suitable anilin dye-stuff, such as nigrosine, dissolved in methyl alcohol, the proportion I use for three gallons of 5 above mixture being one and one-half ounces of nigrosine dissolved in one (1) quart of wood-alcohol. This final composition constitutes my preparatory varnish, and being of about the consistency stated is best applied to the 10 surface of the tanned skin by means of a brush or sponge and to either the flesh side or the grain side, preferably the latter when a goat, kid, or sheep skin is used, and its absorption by or biting effect on the grain-surface 15 of the tanned skin without any roughening or buffing of the latter is almost instantaneous, with the result of forming a homogeneous union therewith having the properties as described, it being understood also that 20 after the preparatory varnish is thus applied, the skin being stretched upon a frame, it is then put into a drying oven or kiln for several hours, or as long as necessary to thoroughly dry it, the heat of the oven being maintained

at about 110° Fahrenheit. Enamel and patent 25 leather is then made therefrom by applying any of the known enamel-varnishes commonly employed as a surface enamel and by the usual drying methods and means.

Having thus described my invention, what 30 I claim as new, and desire to secure by Letters Patent, is—

1. A preparatory varnish for the purpose described, composed essentially of boiled linseed-oil admixed with a solution of guncotton in amyl acetate. 35
2. A mordanting varnish for the purpose described, composed essentially of boiled linseed-oil admixed with a solution of guncotton in amyl acetate, and a coloring-matter 40 dissolved in methyl alcohol.

In testimony whereof I have hereunto affixed my signature this 26th day of December, A. D. 1900.

HARRY C. MCKAY.

Witnesses:

ANDREW V. GROUPE,  
H. T. FENTON.